

Sept. 13, 1960

O. H. THOMAS ET AL

2,952,721

PROCESS FOR ISOMERIZING NORMAL PARAFFINS

Filed Dec. 1, 1958

III. 1.

THE EFFECT OF BORIA ON CATALYST AREA



III. 2.

THE EFFECT OF BORIA ON CATALYST CRUSH STRENGTH

CONDITIONS: 600°F  
1 atm. HCL PARTIAL  
PRESSURE



INVENTORS

John H. Thomas and  
John Goss

BY

James Forward and Leon

ATTORNEYS

2,952,721

**PROCESS FOR ISOMERIZING NORMAL PARAFFINS**

Owen H. Thomas, Chicago, and John Mooi, Park Forest, Ill., assignors to Sinclair Refining Company, New York, N.Y., a corporation of Maine

Filed Dec. 1, 1958, Ser. No. 777,371

14 Claims. (Cl. 260—683.66)

The invention relates to the isomerization of n-paraffinic hydrocarbons to obtain good yields of branched chain aliphatic structures and is particularly concerned with the catalytic isomerization of n-paraffinic hydrocarbons employing a hydrocarbon conversion catalyst. The branched chain aliphatic structures, e.g. isomeric structures of n-paraffins, are particularly useful in providing gasoline components of high octane rating.

In recent years automobile manufacturers have steadily increased the compression ratios of their spark ignition engines as a means of obtaining more power and greater efficiency. As the compression ratios of the engines increase, the hydrocarbon fuel employed must be of higher octane rating to provide efficient knock-free operation notwithstanding that fuel octane rating can be increased through the addition of tetraethyl lead, and other undesirable aspects of engine operation, for instance pre-ignition, can be overcome by the use of other additive components. Thus the problem remains for petroleum refiners to produce higher octane base hydrocarbon fuels under economically feasible conditions.

These refiners now have installed a substantial number of units for reforming straight run petroleum fractions in the presence of free hydrogen and over a platinum metal-alumina catalyst to obtain relatively high octane products. Primarily these products, frequently called reformates, are blended with other gasoline components such as thermal and catalytically cracked gasolines, alkylate, etc., and additives such as tetraethyl lead in obtaining present-day motor fuels. The reforming operation has a number of disadvantages. First, as the octane ratings of the blended engine fuels rise, the octane quality of the reformate must also increase if the blends be otherwise unaltered. This increase results in a substantial reduction in yield particularly in obtaining reformates having octanes (RON neat) of the order of 90 to 95 or above. When the severity of the operation is increased, the platinum metal-containing catalyst becomes fouled more often with carbonaceous deposits which requires more frequent regenerations or replacements. The platinum metal-alumina catalysts are relatively expensive, and either replacement or withdrawal from use during regeneration materially increases the cost of providing a given volume of reformate. These and other factors affecting the yield-octane number-cost relationship make it desirable for the refiner to consider various ways in which high octane hydrocarbon fuel components can be obtained by employing processing methods other than the platinum metal-alumina catalyst reforming operation.

One method now under consideration by petroleum refiners for obtaining stocks of higher octane value involves the isomerization of C<sub>4</sub> or C<sub>5</sub> to C<sub>9</sub> n-paraffinic hydrocarbons, that is n-butane, n-pentane, n-hexane, n-heptane, n-octane, n-nonane and their mixtures with each other and with other hydrocarbons in the same approximate boiling range. In general, as the side chain branching of these n-paraffins increases, their octane ratings rise. A number of catalysts are known as being useful in this

type of operation. An example of such a system is that described in U.S. Patent No. 2,798,105 wherein a platinum-alumina catalyst is employed to isomerize n-butane and n-pentane with the addition of a relatively very small amount in the range of about 0.001 to 0.5% based on the hydrocarbon feed of halogen or a suitable halogen compound. When following this procedure, however, a product containing undesirably large amounts of n-paraffins is produced, the selectivity of the process towards the desired product is low at high conversions and a relatively pure feed is necessary as C<sub>6</sub> paraffins, aromatics and naphthenes are detrimental. Due to the low octane rating of the n-paraffins, a given refiner may not be able to blend the entire product from this isomerization system directly into his gasolines. Rather, under present commercial conditions he will most likely be required to separate the n- and iso-paraffins in the product stream by distillation and then recycle all or a part of the unconverted n-paraffins to the isomerization reaction system.

It is, of course, immediately seen that the decreased yield of isomer structures under the conditions and with the components employed in this process is disadvantageous, and in addition the provision of the required distillation facilities materially adds to the cost of octane enhancement.

However, when following the process of the present invention a sufficiently effective catalytic isomerization process is provided for producing an amount of isomer structures in the product so great that the overall product stream could be used directly in a gasoline pool without requiring distillation for separating the n-paraffins from the product while providing outstanding selectivity towards branched chain structures, for instance, up to 99.0+ volume percent.

In the isomerization process of the present invention C<sub>4</sub> to C<sub>9</sub> n-paraffinic-containing hydrocarbon materials are converted to isomeric structures at relatively intermediate temperatures in the presence of free hydrogen with a hydrocarbon conversion catalyst which is easily regenerable, exhibits good activity as well as good aging characteristics and is stable, with respect to crush strength and surface area, in the presence of a hydrogen halide of atomic weight between about 35 and 85 which is employed in the isomerization reaction. Another highly advantageous feature provided by the use of the hydrocarbon conversion catalyst in this process lay in the obviation of the usual procedure for treating the feeds, employed in processes of this type, to lower the aromatic and naphthene impurities contained therein since the catalyst has a relatively high tolerance limit for these impurities. For instance feeds containing substantial amounts of impurities, e.g. up to about 10 percent aromatics and up to about 20 percent naphthenes can be tolerated as well as feeds usually containing up to about 0.004 percent sulfur. Moreover, as a result of the high isomer content of the resulting product a given refiner may find that it can be blended directly into his gasolines which avoids the necessity for providing distillation facilities to separate the unconverted n-paraffins. However, even if such facilities need to be provided in order to obtain products more concentrated in isomeric structures the process of the present invention still provides increased conversion to branched isomers as compared with others previously available.

Our hydrocarbon conversion catalyst includes catalytically effective amounts of a noble or platinum group metal and boria supported on an alumina base. The catalyst generally contains about 0.01 to 2 weight percent, preferably 0.1 to 1 weight percent, of one or more of the platinum metals of group VIII, that is platinum, palladium, rhodium, ruthenium, osmium or iridium. The small amount of noble metal may be present in the metallic form or as a sulfide, oxide or other combined form. The metal may interact with other constituents of the

catalyst, but if during use the noble metal be present in metallic form then it is preferred that it be so finely divided that it is not detectable by X-ray diffraction means, i.e. that it exists as crystals of less than 50 Angstrom units size. Of the noble metals platinum, palladium and rhodium are preferred.

The boria component is surface dispersible on the support and seems essentially inert to hydrogen halide. It is employed in amounts sufficient to enhance the life of the alumina support and such amounts are, therefore, preferably added in direct proportion to the area of the support. For instance, the amount of boria will usually be about 3 to 20 weight percent, and preferably about 8 to 15 weight percent, of the catalyst. These amounts are particularly effective on alumina having surface areas of about 350 to 600 square meters per gram (BET) before use.

In order for the catalyst to maintain its activity for long periods of time when isomerizing the  $C_4$  to  $C_9$  n-paraffins, it is necessary to provide a hydrogen halide of atomic weight between 35 and 85, e.g. HCl and HBr, during the processing period. The hydrogen halide is added along with or in the n-paraffin feed in an amount of at least about 1 up to about 25 weight percent, based on the hydrocarbon feed, preferably at least about 1% up to about 20%, and advantageously about 5 to 15 weight percent, of the hydrogen halide or of a hydrogen halide-producing material based on the hydrocarbon feed. The addition of the hydrogen halide in these concentrations is continued over the processing period in order to maintain an adequate concentration of this component and insure the stability of the catalyst against undue aging. The hydrogen halide can be added separately to the reaction system, in the hydrogen-containing recycle gases or in the n-paraffin feedstock.

Instead of supplying the hydrogen halide with an atomic weight between 35 and 85 as such, an organo-halogen compound or other substance which will produce the hydrogen halide under the isomerization conditions can be employed. Suitable hydrogen halide precursors of this type include the elemental halogens, chlorine and bromine; mono- and polyhalo-alkanes such as carbon tetrachloride, chloroform and tertiary butyl chloride; or other available materials which will be converted under the conditions of isomerization to obtain the desired amount of hydrogen halide.

The noble metal and boria constituents of the catalyst are deposited on an absorptive alumina base of the activated or calcined type. The base is usually the major component of the catalyst, generally constituting at least about 75 weight percent on the basis of the catalyst, preferably at least about 80 to 90%. The catalyst base is an activated or gamma-alumina such as those derived by calcination of amorphous hydrous alumina, alumina monohydrate, alumina trihydrate or their mixtures. The catalyst base precursor most advantageously is a mixture predominating, for instance about 65 to 95 weight percent, in one or more of the alumina trihydrates bayerite I, bayerite II (randomite) or gibbsite, and about 5 to 35 weight percent of alumina monohydrate (boehmite), amorphous hydrous alumina or their mixture. The alumina base can contain small amounts of other solid oxides such as silica, magnesia, natural or activated clays (such as kaolinite, montmorillonite, halloysite, etc.), titania, zirconia, etc., or their mixtures. Although the components of the catalyst can vary as stated, a preferred catalyst contains platinum and boria deposited on activated alumina.

The isomerization reaction conditions used in the method of the present invention include a temperature sufficient to maintain the n-paraffin feed in the vapor phase under the pressure employed. Generally, this temperature will be from about 500 to 800° F., preferably about 575 to 650° F., while the pressure will be superatmospheric for instance ranging from about 200 to 1000 p.s.i.g.,

preferably about 300 to 600 p.s.i.g. The catalyst can be used as a fixed, moving or fluidized bed or in any other convenient type of handling system. The fixed bed system seems most advantageous at this time and the space velocity will in most cases be from about 0.25 to 8:1, preferably about 0.75 to 4:1, weights of n-paraffin per weight of catalyst per hour (WHSV).

Free molecular hydrogen must be present in our reaction system and the hydrogen to n-paraffin molar ratio will usually be from about 0.01 to 20:1 or more, preferably about 2 to 10:1. Conveniently, the hydrogen concentration is maintained by recycling hydrogen-rich gases from the reaction zone. These gases will usually contain hydrogen halide at least after the initial processing period and as there is usually only a small loss of the halide at processing conditions, the desired concentration in the feed may be maintained merely by recycling the hydrogen-hydrogen halide-containing gases with a small make-up of hydrogen halide.

As previously stated the preferred catalyst base material is an activated or gamma-alumina made by calcining a precursor predominating in alumina trihydrate. An alumina of this type is disclosed in U.S. Patent No. 2,838,444. The alumina base is derived from a precursor alumina hydrate composition containing about 65 to 95 weight percent of one or more of the alumina trihydrate forms, gibbsite, bayerite I and bayerite II (randomite) as defined by X-ray diffraction analysis. The substantial balance of the hydrate is amorphous hydrous or monohydrate alumina. Trihydrates are present as well defined crystallites, that is they are crystalline in form when examined by X-ray diffraction means. The crystallite size of the precursor alumina trihydrate is relatively large and usually is in the 100 to 1000 Angstrom unit range. The calcined alumina has a large portion of its pore volume in the pore size range of about 100 to 1000 Angstrom units generally having about 0.1 to about 0.5 and preferably about 0.15 to about 0.3 cc./g. of pore volume in this range. As described in the patent the calcined catalyst base can be characterized by large surface area ranging from about 350 to about 550 or more square meters/gram when in the virgin state as determined, for example, by the BET adsorption technique. A low area catalyst base prepared by treating the predominantly trihydrate base precursor is described in U.S. Patent No. 2,838,445. This base when in the virgin state has substantially no pores of radius less than about 10 Angstrom units and the surface area of the catalyst base is less than about 350 square meters/gram and most advantageously is in the range of about 150 to 300 square meters/gram.

The platinum group metal component of the catalyst can be added to the alumina base by known procedures. For instance, the platinum metal component can be deposited on a calcined or activated alumina, but it is preferred to add the platinum metal component to the alumina hydrate precursor. Thus platinum can be added through reaction of a halogen platinum acid, for instance, fluoro-, chloro-, bromo- or iodo-platinic acid, and hydrogen sulfide in an aqueous slurry of the alumina hydrate. The hydrogen sulfide can be employed as a gas or an aqueous solution. Alternatively, the platinum component can be provided by mixing an aqueous platinum sulfide sol with the alumina hydrate. This sol can be made by reaction in an aqueous medium of a halogen platinic acid with hydrogen sulfide. The alumina hydrate containing the platinum metal can be dried and calcined usually at a temperature from about 750 to 1200° F. or more to provide the activated or gamma-alumina modifications. The boria can be added to the catalyst in any stage of its preparation. It may be incorporated in the support, for instance, by precipitation, coprecipitation, impregnation, and mulling either before or after the addition of the group VIII metal. It can also be applied by impregnation from solution

(water, organic or inorganic solvents) or from a gas phase. However, it is frequently added to the catalyst after it has been formed by tableting or extrusion and calcined. After the boria is added in this procedure the catalyst can be recalcined.

The catalyst of the present invention can be easily regenerated employing conventional procedures, for instance by subjecting it to an oxygen-containing gas at temperatures sufficient to burn off carbon deposited on the catalyst during the conversion of petroleum hydrocarbon feedstock. This oxygen-containing gas, e.g. an oxygen-nitrogen mixture, can contain about 0.01 weight percent to 5 weight percent oxygen but preferably contains about 0.5 to 1.5 weight percent oxygen and is introduced at a flow rate such that the maximum temperature at the site of combustion is below about 1000° F.

When following the process of the present invention, outstanding selectivity, as an example, as high as 99+%, and good conversions of n-paraffinic hydrocarbon materials to corresponding isomeric structures are provided. For instance, the conversion of n-pentane to isopentane is generally about 50 to 70 percent and usually above about 60% based on the pentane feed; about 60 to 85 percent, usually above about 75 percent, of n-hexane is converted to iso-hexane including about 6 to 20 percent of 2,2-dimethylbutane, a high octane component; and about 35 to 50 percent, usually above about 42 percent, of n-butane is converted to isobutane.

The paraffinic feed material employed in our process is generally a C<sub>4</sub> to C<sub>9</sub> n-paraffinic-containing cut derived from crude petroleum hydrocarbons, as by distillation, reforming and extraction processes. The feed we prefer to use, however, is a blend of n-pentane and n-hexane usually containing about 25 percent or more of n-hexane and preferably a predominant amount of n-hexane.

The following specific examples will serve to illustrate our invention but they are not to be considered limiting.

#### EXAMPLE I

##### (A) Preparation of noble metal alumina composition

A noble metal alumina composition of the kind described in U.S. Patent No. 2,838,444 can be employed in preparing the catalyst used in the process of our invention. The composition of this patent can be made as follows. Pure aluminum metal is dissolved in pure hydrochloric acid, and the resulting solution is mixed with deionized water to form an aqueous aluminum chloride solution and an alumina gel is prepared equivalent to approximately 65 grams of Al<sub>2</sub>O<sub>3</sub> per liter. A separate deionized water solution of NH<sub>4</sub>OH is prepared containing approximately 65 grams of ammonia per liter. These two reagents in approximate volume ratio of 1:1 are intimately mixed as a flowing stream at a pH of 8.0. The flowing stream is passed to a stoneware container and an alumina hydrate is visible. The precipitated hydrate is filtered from the mother liquid and washed to <0.2% chloride by successive filtrations and reslurrys in deionized water until the desired chloride concentration is reached. In each reslurrying ammonia is added to give a pH of about 9. The washed hydrate is covered with water in a container and aged at about 90° F. until it is approximately 70% trihydrate, the remaining being substantially of the amorphous or monohydrate forms. The total hydrate composition is comprised of 42% bayerite, 18% randomite, 11% gibbsite, 20% boehmite, and 9% amorphous as determined by X-ray diffraction analysis. The aged hydrate is mixed with deionized water in a rubber-lined container to provide a slurry of about 7 weight percent Al<sub>2</sub>O<sub>3</sub> at a pH of about 8.0. A chloroplatinic acid solution in deionized water (0.102 gram platinum per milliliter) is stirred into the slurry and the slurry is then contacted with a deionized water solution which has been saturated with H<sub>2</sub>S at 78° F. to precipitate the platinum.

The pH of the slurry is adjusted to 6.0 to 6.5 by ammonium hydroxide addition and the solids of the slurry are dried on a horizontal drum drier to give a powder of generally less than 20 mesh. The drum dried powder is mixed in a planetary type dough beater with sufficient deionized water to indicate 26 weight percent water on a Central Scientific Company infra-red moisture meter containing a 125 watt bulb, cat. No. 26675. The resulting mixture is forced through a die plate having holes  $\frac{1}{16}$ " in diameter bolted to a 3 $\frac{1}{2}$ " Welding Engineers screw extruder. The resulting strands are broken to particles of length varying generally between about  $\frac{1}{16}$ " to 1".

The particles are dried at 230° F. and calcined by heating to 925° F. in a flow of nitrogen gas followed by a flow of air while the composition is maintained at a temperature in the range of 865° to 920° F. The composition thus produced analyzes about 0.6 weight percent of platinum which is in sufficiently divided form so as to exhibit by X-ray diffraction studies the substantial absence of crystallites or crystals of size larger than 50 Angstrom units. After the calcination the composition has an area (BET method) within the range from about 350 to 550 square meters/gram.

##### (B) Preparation of noble metal-boria-alumina catalyst

A platinum-alumina composition prepared essentially as described above, except that air was used for the complete calcination procedure, and containing about 0.6% platinum was employed in preparing the noble metal-boria-alumina catalyst by the following procedure. 300 grams of the calcined platinum-alumina composition were weighed into a 6" crystallizing dish. 59 grams of H<sub>3</sub>BO<sub>3</sub> were dissolved in 279 ml. of deionized water by heating to boiling. The hot boric acid solution was poured over the catalyst and stirred thoroughly with a rubber spatula. The catalyst was placed in a forced air drying oven, set at 284° F. for 4 hours. The catalyst was stirred occasionally while drying. The oven dried catalyst was transferred to a saggar and placed in a muffle furnace preheated to 1000° F. The catalyst was held at 1000° F. for 2 hours and cooled in a desiccator. Analysis: 9.95% B<sub>2</sub>O<sub>3</sub>.

##### (C) Activation of noble metal-boria-alumina catalyst

Although the noble metal-boria-alumina catalyst can be activated during isomerization processing on stream, it can be pre-reduced or pre-activated. Pre-activation can be accomplished by treatment with hydrogen at an elevated temperature, for instance about 800 to 1000° F. Rather than pre-activate the catalyst it can be used directly in the isomerization process and the presence of the free hydrogen gas will cause activation in the initial stages of the process.

An example of pre-activation follows: 40 grams of this catalyst were supported on glass beads in the center of a 1-inch I.D. Universal stainless steel reactor. The reactor was set in place in a bronze-block furnace controlled by "Microswitch" thermostats. The catalyst was heated to 800° F. under atmospheric pressure of pure hydrogen flowing at about 2 cu. ft./hr. These conditions were maintained for 16 hours. At this time the reactor is cooled to operating temperatures and reaction conditions are established for processing the paraffin feed.

#### EXAMPLE II

The isomerization process of the present invention is illustrated by runs A, B, C and D (presented below in Table I) employing platinum, palladium, rhodium and platinum, respectively, as the group VIII metal. In addition, run E employing the boria-alumina catalyst without the group VIII metal is provided for comparison purposes. All runs were conducted under the conditions specified above and the catalysts were prepared essentially according to the procedure as described in Example I except in the preparation of the catalyst used in run E,

where the group VIII metal was omitted. The results of these runs are also presented in this table. The yields in weight percent of the isomeric structures in this table and throughout the specification are based on the corresponding total pentane and hexane structures present in the feed.

cyclopentane plus cyclohexane is fed to a reactor unit containing platinum-boria-alumina catalyst, prepared essentially as described in Example I(B) above, with a Ruska pump while the  $H_2$ -HCl was fed in by means of a  $H_2$ -HCl blend (5 mole percent HCl). The conditions were  $625^\circ F.$ , 300 p.s.i.g., 5/1  $H_2$ /HC, 1 WHSV,

TABLE I

| Run.                                                | 971-20<br>A          | 971-11<br>B          | 971-28<br>C          | 971-13<br>D                                                               | 971-29B<br>E                   |
|-----------------------------------------------------|----------------------|----------------------|----------------------|---------------------------------------------------------------------------|--------------------------------|
| Catalyst:                                           |                      |                      |                      |                                                                           |                                |
| Number.....                                         | 480-279              | 480-326              | 480-319              | 0.6% Pt, 10% B <sub>2</sub> O <sub>3</sub> Al <sub>2</sub> O <sub>3</sub> | 480-316, 10% boria on alumina. |
| Description.....                                    | Pt-boria on alumina. | Pd-boria on alumina. | Rh-boria on alumina. | (1).....                                                                  | (2).....                       |
| Feed:                                               |                      |                      |                      |                                                                           |                                |
| Conditions:                                         |                      |                      |                      |                                                                           |                                |
| Temperature, ° F.....                               | 600                  | 600                  | 600                  | 600                                                                       | 600                            |
| WHSV.....                                           | 1.0                  | 1.0                  | 1.0                  | 1.0                                                                       | 1.0                            |
| Pressure, p.s.i.g.....                              | 300                  | 300                  | 300                  | 300                                                                       | 300                            |
| $H_2$ /HC (mole ratio).....                         | 5.0                  | 5.0                  | 5.0                  | 5.0                                                                       | 5.0                            |
| HCl (weight percent based on hydrocarbon feed)..... | 12.5                 | 5                    | 5                    | 12.5                                                                      | 12.5+                          |
| Yields (weight percent):                            |                      |                      |                      |                                                                           |                                |
| i-C <sub>5</sub> .....                              | 61.5                 | 60.3                 | 62.6                 | 62.1                                                                      | 8.4                            |
| i-C <sub>6</sub> .....                              | 79.9                 | 79.3                 | 79.4                 |                                                                           |                                |
| 2,2-DMB.....                                        | 8.4                  | 13.9                 | 13.4                 |                                                                           |                                |
| Selectivity, C <sub>5</sub> + weight percent.....   | 96.2                 | 99.0                 | 98.7                 | 99                                                                        | 99.0+                          |

## Feed:

(1) Phillips Commercial Grade n-C<sub>5</sub>-C<sub>6</sub> blend:

Composition:  
 8.8% i-C<sub>5</sub>; 30.6% n-C<sub>5</sub>;  
 8.1% 2,3-DMB+2-MP;  
 9.5% 3-MP; 36.7% n-C<sub>6</sub>;  
 11.5% MCP; 9% CyC<sub>6</sub>;  
 2.9% benzene and 0.0034% sulfur.

(2) Phillips Pure Grade n-C<sub>5</sub>+0.4 wt. percent n-amyl chloride.

## EFFECT OF BORIA ON THE ALUMINA STRUCTURE

The superior characteristics, in the presence of the hydrogen chloride component in the isomerization process of the present invention, of a platinum-boria-alumina composition prepared essentially according to the procedure as described in Example I above is shown below in comparison with a platinum-alumina composition without the boria and prepared essentially as described in Example I(A) above.

A 5.46 gram portion of commercial Sinclair-Baker RD-150 catalyst (a platinum-alumina catalyst prepared essentially according to the procedure described in Example I(A) above) was placed in a Pyrex tube. The catalyst was supported on a sintered glass disk to allow gas to pass up through it. A thermocouple well was led from the side of the tube into the catalyst bed. Anhydrous hydrogen chloride gas was passed through the catalyst at a rate of about 25 cc./min. at atmospheric pressure. A furnace was placed around the tube, heat was turned on and the temperature inside the thermowell brought to  $600^\circ F.$  The temperature was maintained at  $600 \pm 10^\circ F.$  for 188 hours. The catalyst was purged of HCl with flowing  $H_2$  for two hours, cooled and removed from the tube.

A 7.00 g. portion of Sinclair-Baker RD-150 catalyst+10% B<sub>2</sub>O<sub>3</sub> (480-279), was charged to a similar apparatus and treated in an identical manner as Sinclair-Baker RD-150 catalyst described in the previous paragraph. The surface area of each catalyst was determined before and after this treatment. The measurement was made by the BET method using N<sub>2</sub> adsorption at the temperature of liquid nitrogen. The Sinclair-Baker RD-150 catalyst area fell from 500 to 180 square meters/gram while the Sinclair-Baker RD-150-B<sub>2</sub>O<sub>3</sub> catalyst area fell from 380 to 280 square meters/gram. The results indicate that B<sub>2</sub>O<sub>3</sub> has a beneficial effect on the alumina structure.

## IMPURITY TOLERANCE LIMIT

The relatively high tolerance limit of a platinum-boria-alumina catalyst for the aromatic and naphthalene contaminants in n-paraffinic-containing hydrocarbon feeds employed in an isomerization process is demonstrated below.

A Phillips commercial grade n-C<sub>5</sub>-C<sub>6</sub> blend (35-65) containing 4% aromatics and 16 weight percent methyl-

35 12.5 weight percent HCl based on hydrocarbon feed. The product was collected by means of Dry Ice-acetone cooling of a product recovery flask. The product yields were 64% i-C<sub>5</sub>, 80% total i-C<sub>6</sub>, 14% 2,2-dimethylbutane. The C<sub>5</sub>+ selectivity was approximately 98 weight percent.

## EFFECT OF BORIA ON AREA, CRUSH STRENGTH AND SELECTIVITY

40 A charge of platinum-boria-alumina catalyst, prepared essentially as described in Example I above and containing 0.6% platinum and 10% boria, was tested in a gas reactor unit under a variety of processing conditions. Periodic activity checks were taken throughout the testing 45 period. Between intervals of hydrocarbon processing the catalyst was blocked in the reactor under a  $H_2$ -HCl atmosphere at reaction temperature and pressure. The catalyst was subjected to 900 hours of HCl contact and 160 hours of noncontinuous hydrocarbon processing under 50 conditions including  $600^\circ F.$ , 300 p.s.i.g., 5/1  $H_2$ /HC, 1 WHSV, 12.5 weight percent HCl and using a Phillips commercial grade blend of C<sub>5</sub> and C<sub>6</sub>. A similar evaluation was conducted using Sinclair-Baker RD-150 catalyst. A summary of the area and crush strength results 55 are presented in Figures 1 and 2, respectively.

56 A similar platinum-boria-alumina catalyst composition after 430 hours of continuous contact with HCl in a glass flow system gave the following results for hydrocarbon processing.

## 60 Conditions:

600° F., 1 WHSV, 5/1H<sub>2</sub>/HC, 300 p.s.i.g., 12.5 weight percent HCl, Phillips C.G. C<sub>5</sub>-C<sub>6</sub> blend.

## Yields:

65 i-C<sub>5</sub>..... 65.3  
 Total i-C<sub>6</sub>..... 79.7  
 2,2-DMB..... 14.5  
 C<sub>5</sub>+ selectivity..... 97.7

70 There can be no doubt of the beneficial effect of boria when one compares this result with that obtained for RD-150 after a similar 430 hour treatment with HCl.

## Conditions:

600° F., 1 WHSV, 5/1H<sub>2</sub>/HC, 300 p.s.i.g., 12.5 weight percent HCl, Phillips C.G. C<sub>5</sub>-C<sub>6</sub> blend.

## Yields:

|                              |      |
|------------------------------|------|
| i-C <sub>5</sub>             | 63.5 |
| Total i-C <sub>6</sub>       | 76.8 |
| 2,2-DMB                      | 10.0 |
| C <sub>5</sub> + selectivity | 65.1 |

In addition to its loss in isomerization selectivity, RD-150 crushing strength after 430 hours of HCl contact (2.1 lbs.) is decreased to zero after only 17 hours of hydrocarbon processing. These results emphasize the inability of RD-150 alone to function catalytically in the presence of HCl.

## PROCESS AGING CHARACTERISTICS

A charge of platinum-boria-alumina catalyst, prepared essentially as described in Example I above and containing 0.6% platinum and 10% boria, was tested for aging characteristics in a reactor unit. A Phillips commercial grade n-pentane:n-hexane blend (a 32 volume percent n-pentane:68 volume percent n-hexane blend) including 3.2 percent aromatics and 14 percent C<sub>6</sub> naphthenes was conducted to the reactor under conditions (run 14-192) including 600° to 605° F., 600 p.s.i.g., 5/1 mol ratio of H<sub>2</sub>+HCl/HC recycle, 0-0.6/1 mol ratio of H<sub>2</sub>+HCl/HC make-up, and 1 WHSV. The H<sub>2</sub>+HCl/HC make-up was initially employed at a molar ratio of 0.6/1 with the H<sub>2</sub> containing 5 mol percent HCl, at 550 hours substantially pure hydrogen was substituted as the make-up at the same ratio, at 690 hours the ratio was switched to 0.3/1 with the H<sub>2</sub> containing 5 mol percent HCl, and at 1020 hours the ratio was switched to 0.6/1. This data shows no apparent loss in activity after 1350 hours of processing.

TABLE II

| Yields (weight percent):                     |      |      |       |       |
|----------------------------------------------|------|------|-------|-------|
| i-C <sub>5</sub> yield                       | 61.2 | 62.9 | 63.5  | 63.5  |
| i-C <sub>6</sub> yield                       | 74.5 | 79.8 | 78.2  | 78.2  |
| 2,2-DMB yield                                | 12.5 | 12.6 | 13.0  | 13.0  |
| C <sub>5</sub> + selectivity, weight percent | 96   | 95   | 95    | 94    |
| Hrs. on stream                               | 115  | 525  | 1,035 | 1,350 |

It is claimed:

1. In a method of isomerizing a C<sub>4</sub> to C<sub>9</sub> n-paraffinic-containing hydrocarbon feed, the step comprising contacting said feed in the vapor phase with a catalyst at a temperature of about 500 to 800° F., superatmospheric pressure, and in the presence of free hydrogen and while providing about 1 to 25% of a hydrogen halide based on said feed, said catalyst consisting essentially of about 0.01 to 2% of a platinum group noble metal and about 3 to 20% of boria supported on an activated alumina.
2. The method of claim 1 in which the catalyst contains about 0.1 to 2% of the platinum group metal.
3. The method of claim 1 in which the temperature is about 575 to 650° F. and the feed contains n-pentane and n-hexane.
4. The method of claim 1 in which the noble metal is selected from the group consisting of platinum, palladium and rhodium, and is about 0.1 to 1% of the catalyst, the boria is about 8 to 15% of the catalyst and the hydrogen halide is hydrogen chloride.
5. The method of claim 1 in which the activated alu-

mina is derived by calcination of an alumina hydrate precursor consisting essentially of about 65 to 95% of alumina trihydrate and about 5 to 35% of a member selected from this group consisting of amorphous hydrous alumina, alumina monohydrate and their mixture, and the activated alumina has an area of about 350 to 550 square meters per gram before use.

6. The method of claim 3 in which the feed contains substantial amounts of aromatic and naphthenic impurities.

7. The method of claim 1 in which the temperature is about 575 to 650° F. and the noble metal is platinum and is about 0.1 to 1.0% of the catalyst, the boria is about 8 to 15% of the catalyst, the hydrogen halide is hydrogen chloride, and the activated alumina is derived by calcination of an alumina hydrate precursor consisting essentially of about 65 to 95% of alumina trihydrate and about 5 to 35% of a member selected from the group consisting of amorphous hydrous alumina, alumina monohydrate and their mixture, and has an area of about 350 to 550 square meters per gram before use.

8. The method of claim 7 in which the feed contains n-pentane and n-hexane blend.

9. The method of claim 1 wherein the catalyst is prepared by contacting a calcined platinum metal alumina composition with a heated aqueous solution of boric acid and calcining the resulting platinum metal-boria-alumina composition.

10. The method of claim 4 wherein the catalyst is prepared by contacting a calcined platinum metal alumina composition with a heated aqueous solution of boric acid and calcining the resulting platinum metal-boria-alumina composition.

11. The method of claim 1 in which the noble metal is selected from the group consisting of platinum, palladium and rhodium and is about 0.1 to 2 percent of the catalyst, and the boria is about 8 to 20 percent of the catalyst.

12. The method of claim 11 wherein the catalyst is prepared by contacting a calcined platinum metal-alumina composition with a heated aqueous solution of boric acid and calcining the resulting platinum metal-boria-alumina composition.

13. The method of claim 1 wherein the noble metal is selected from the group consisting of platinum, palladium and rhodium and is about 0.1 to 2 percent of the catalyst, and the boria is about 3 to 15 percent of the catalyst.

14. The method of claim 13 wherein the catalyst is prepared by contacting a calcined platinum metal-alumina composition with a heated aqueous solution of boric acid and calcining the resulting platinum metal-boria-alumina composition.

## References Cited in the file of this patent

## UNITED STATES PATENTS

|           |                  |               |
|-----------|------------------|---------------|
| 2,751,333 | Heinemann        | June 19, 1956 |
| 2,798,105 | Heinemann et al. | July 2, 1957  |
| 2,831,908 | Starnes et al.   | Apr. 22, 1958 |
| 2,834,740 | Johnson et al.   | May 13, 1958  |
| 2,838,444 | Teter et al.     | June 10, 1958 |